

1

3,505,095

## PREPLATING TREATMENT FOR MARAGING STEELS

George S. Petit and Ralph R. Wright, Oak Ridge, Tenn., assignors to the United States of America as represented by the United States Atomic Energy Commission  
No Drawing. Filed Apr. 5, 1967, Ser. No. 628,790

Int. Cl. B44d 1/092

U.S. Cl. 117—50

4 Claims

### ABSTRACT OF THE DISCLOSURE

The coating of maraging steels, i.e., low carbon steels containing about 17 to 25 weight percent nickel, 3 to 5 weight percent molybdenum, and small percentages of cobalt, aluminum, and titanium, with a protective metal plate has been hampered by the formation of a layer of black smut on the steel surfaces during preplating pickling operations. This smut is believed to be due to the presence of a molybdenum compound on the steel surfaces that is removed by contacting the affected surfaces with an aqueous solution of lactic acid and hydrogen peroxide.

The present invention relates generally to treating low carbon maraging steels for reception of protective plating, and more particularly to the preparation of the surfaces of such steels by removing a layer of black smut which interferes with the adhesion of nickel plating with the steels. This invention was made in the course of, or under, a contract with the U.S. Atomic Energy Commission.

It has been recognized for some time that maraging steels possess unique properties which render the use of such steels particularly desirable in applications where strength and toughness are of major importance, such as, for example, in the fabrication of liquid centrifuge rotors or bowls, bearings, shafts, tubulations, seals, etc. Maraging steel is an iron-nickel alloy composed primarily of 17 to 25 weight percent (w/o) nickel, about 3 to 5 w/o molybdenum, about 6 to 9 w/o cobalt, less than about 0.03 w/o carbon, fraction percentages of titanium and aluminum, and the balance essentially iron. This type steel is a high-strength alloy possessing good ductility, exceptional toughness, and develops a martensitic structure and its high-strength properties by annealing at elevated temperatures, e.g., about 500° C. for a period of several hours.

While maraging steel possesses the desired properties of high strength and toughness, it is subject to wear and also to corrosion by solutions such as cesium chloride which may be employed in centrifuge operations. This shortcoming of maraging steel is readily overcome by providing the steel with a protective coating of metal such as nickel, which may be applied by electroplating or by non-electrolytic means.

Normally, the procedure for applying a protective metal coating, e.g., a nickel plate, to a base metal requires that the surface of the latter be first conditioned in such a manner that the nickel plate tightly bonds to the base metal when deposited by an electroplating operation or by an electroless plating bath. This surface preparation is somewhat conventional and includes the removal of gross contaminants such as rust, oxide, scale, grease, and the like by employing solvents or scouring powders for the removal of the grease and acid pickling baths for the removal of the other contaminants. In addition to the removal of the contaminants, the acid pickling bath also etches or slightly roughens the surface of the base metal to make the base metal more likely to provide a good bond with the nickel plate. However, it was found that

2

maraging steel, when heat treated prior to final machining to give the metal its desirable strength properties, was not receptive to nickel plating in that the nickel plating was either prevented from depositing on the maraging steel or, if deposited, did not adequately bond with the steel. This peculiar trait of maraging steel was found to be due to the formation of a velvety layer of a black smut-like substance on the steel surface during the acid pickling operation. It is believed that this smut is a molybdenum compound, perhaps a form of molybdenum oxide, which forms on the surface of the maraging steel when heat treated possibly because the heat treating step causes molybdenum to migrate to the surface.

Efforts to remove or otherwise compensate for the smut formation have not been entirely successful. For example, the modification of conventional pretreating baths by pickling with a chloride-acid "activator," e.g., a hydrochloric acid solution, has not provided satisfactory results. Another unsuccessful effort to improve the bonding of the nickel plating involved the use of an electro-strike coating in a nickel chloride-hydrochloric acid solution. It has been suggested that an anodic-type pretreatment using a bath of sulfuric acid with a small addition of hydrofluoric acid would provide a solution to the smut problem. However, the use of hydrofluoric acid would be objectionable since the surface of the maraging steel article would be attacked excessively so as to render it extremely difficult to provide the surface finish necessary for applications requiring smooth surfaces. Further, with maraging steel articles of relatively complex shapes in that configurations such as corners, threads, surface protuberances, sharp angles, and the like may be present, the use of anodic treatments is not desirable since the high current densities encountered in such areas may produce excessively large diametral changes in the article so as to render it unacceptable for its intended purpose. Another disadvantage to using anodic treatments is due to the fact that such treatments require that the cathode have a configuration similar to that of the steel article being treated. Also, such anodic treatments are somewhat time-consuming and relatively expensive.

It is, therefore, the aim of the present invention to minimize or obviate the above and other shortcomings or drawbacks previously suffered in providing maraging steels with a protective metal coating such as nickel. This goal is achieved by contacting maraging steel articles with an aqueous solution of lactic acid and hydrogen peroxide. This treatment prepares the article surface for reception of an adherent metal coating by converting the smut to a compound which is readily dissolved in the solution.

An object of the present invention is to render maraging steel surfaces acceptable for receiving an adherent coating of nickel or another suitable metal.

Another object of the present invention is to provide a treatment for maraging steel surfaces which is applicable after the conventional contaminant removal to produce a surface free of smut for facilitating the application and bonding of nickel coatings.

Generally, the present invention involves the employment of a unique surface treatment for maraging steel that has been found to be capable of removing or otherwise rendering ineffective a layer of a molybdenum compound which heretofore prevented metal coatings from tenaciously adhering with the steel. As briefly mentioned above, the molybdenum compound (composition unknown) is believed to be formed on the surface of maraging steel articles during the heat treatment operation required to provide the steel with its desired strength properties. This molybdenum compound appears on the surface of the maraging steel as a uniform and continuous layer or coating and has the appearance of a some-

what velvet-like black smut after the steel has been subjected to acid pickling treatments.

The above-mentioned unique treatment consists of an aqueous solution or bath of lactic acid and hydrogen peroxide that "de-smuts" the exposed surface of the maraging steel by oxidizing the molybdenum compound to a higher valence state and then converting this compound to a complex of an unknown composition that is readily dissolved in the aqueous solution. This smut removing solution preferably consists of about 10 to 20 percent (volume) lactic acid, about 5 to 10 percent (volume) of 30-percent hydrogen peroxide, and the balance water. The smut removal is usually accomplished by dipping or immersing the smut carrying maraging steel article into the treating solution after completing the conventional degreasing and pickling treatments for a duration of about 2 minutes with the solution at room temperature. Upon completing the de-smutting operation the steel article is preferably thoroughly rinsed in distilled or de-ionized water to assure minimal transfer of impurities into the plating bath.

By utilizing the de-smutting treatment of the present invention together with the conventional degreasing and pickling treatments the maraging steel articles are provided with a "clean" surface to which nickel and other metal coatings tightly bond. The particular procedure for applying the metal coating is not critical in that conventional electroless plating baths or electroplating procedures may be readily employed. Further, while this invention relates primarily to the coating of maraging steel with nickel, it is to be understood that coatings of other metals such as copper, silver, gold, etc., may be adequately bonded to maraging steel by practicing the present invention.

Inasmuch as a highly uniform plating is desirable for applications such as centrifuge rotors, it may be desirable to use a pickling treatment which is capable of providing minimal surface roughness on the maraging steel articles. For example, a machined article having a surface roughness of approximately 8 microinches exhibits a surface roughness of about 13 microinches after cleaning and plating when the pickling solution is composed of 400 grams of  $\text{Al}(\text{NO}_3)_3 \cdot 9\text{H}_2\text{O}$  and 400 milliliters 38% HCl diluted to one liter with water. Pickling in this solution may be achieved in about 2 to 5 minutes with the solution at a temperature of 42° C. On the other hand, where such surface uniformity is not necessary, a cleaning and pickling solution of concentrated (38%) HCl with about 5 percent (volume) of 30% hydrogen peroxide may be employed. Plated articles using this treatment together with a degreaser and the de-smutting solution of this invention have a surface roughness of about 40 to 80 microinches.

In order to provide a better understanding of the invention, an example of a typical preplating treatment of a maraging steel article is set forth below. This example is merely illustrative and is not intended to limit the invention to the particular degreasing and pickling agents, plating material, or the sequence and duration of the various treating steps.

A centrifuge rotor of maraging steel heat treated and machined to the desired dimensions is first scrubbed with a commercially available scouring powder to remove some of the gross contaminants and washed thoroughly with tap water. The rotor is then vapor degreased with trichloroethylene and thereafter immersed for a period of 4 minutes in a pickling solution consisting essentially of 400 grams of  $\text{Al}(\text{NO}_3)_3 \cdot 9\text{H}_2\text{O}$  and 400 milliliters of 38-percent HCl diluted to one liter with water. The solution is maintained at 42° C. After completing the pickling treatment the rotor is rinsed with tap water and then immersed for a period of 2 minutes in the de-smutting solu-

tion consisting essentially of 15 percent lactic acid, 8 percent hydrogen peroxide, and the balance water. The de-smutting solution is preferably maintained at room temperature. The rotor is then rinsed in distilled water to complete the preparation necessary to receive and bond with a nickel plate of desired thickness that may be subsequently applied in any desired manner.

It will be seen that the present invention sets forth a significant improvement in the art for providing maraging steels with protective metal plating or coatings in that the unique cleaning treatment of this invention assures that the bond of the plate to the surface of the maraging steel is not affected by the molybdenum compound (smut) heretofore found highly deleterious to the bond. Another advantage is that maraging steels can be provided with soundly bonded metal coatings without concern as to whether or not the maraging steel had been previously heat treated. Further, while the invention is primarily concerned with the treatment of maraging steels, it is to be understood that the other steels and alloys which suffer from the presence of the molybdenum compound on their surfaces may be similarly treated and plated with satisfactory results. Additionally, maraging steels and other metals may have some of the undesirable molybdenum compound on surfaces thereof regardless of whether or not the metal has been subjected to heat treatments. Consequently, the surface treatment of the present invention is also applicable to non-heat treated metals, since the removal of even trace amounts of the bond-resisting compound from the metal surface results in the establishment of a better bond between the coating material and the base metal.

What is claimed is:

1. The method of improving the bonding properties of protective metal coatings to a molybdenum containing metal having surfaces thereof coated with a layer of a bond-resisting molybdenum compound, comprising the treating of the molybdenum containing metal prior to the application of the metal coating by contacting said surfaces thereof with an aqueous solution containing as essential ingredients lactic acid and hydrogen peroxide.
2. The method claimed in claim 1, wherein the solution consists essentially of about 10 to 20 volume percent lactic acid, about 5 to 10 volume percent of 30-percent hydrogen peroxide, and the balance water.
3. The method claimed in claim 2, wherein the metal is contacted with the solution for a period of about 2 minutes.
4. The method claimed in claim 3, wherein the metal is a steel alloy consisting essentially of 17 to 25 weight percent nickel, about 3 to 5 weight percent molybdenum, about 6 to 9 weight percent cobalt, less than about 0.3 weight percent carbon, fractional weight percentages of titanium and aluminum, and the balance iron.

#### References Cited

##### UNITED STATES PATENTS

- |           |        |                   |            |
|-----------|--------|-------------------|------------|
| 3,029,158 | 4/1962 | Lee et al. -----  | 117—50     |
| 3,147,154 | 9/1964 | Cole et al. ----- | 117—130 XR |
| 3,386,896 | 6/1968 | Finne -----       | 117—50 XR  |

##### OTHER REFERENCES

- Downey, T. A., Organic Acids in Metal Cleaning and Finishing, In Metal Finishing, vol. 60, No. 10, October 1962, pages 50—57 and 65.

ALFRED L. LEAVITT, Primary Examiner

JANYCE A. BELL, Assistant Examiner

U.S. CL. X.R.

117—49, 130; 156—3; 204—32; 252—79, 1, 81